

1

2,830,024

## EXTREME PRESSURE GEAR LUBRICANT

Paul R. Chapman, Crystal Lake, and Allan A. Manteuffel, Union, Ill., assignors to The Pure Oil Company, Chicago, Ill., a corporation of Ohio

No Drawing. Application September 9, 1953  
Serial No. 379,285

3 Claims. (Cl. 252—46.7)

The present invention relates to lubricating compositions having extreme pressure characteristics with improved storage stability and good performance characteristics and, more particularly, it relates to lubricants for gears, such as hypoid gears, transmissions, and differentials.

It is known to prepare extreme pressure additives for use in lubricating oil compositions which have the ability of imparting to the lubricating composition resistance to sudden heavy (shock) loading conditions in metal-to-metal working parts or prolonged heavy loading as in metal working operations, such as cutting, deep drawing, and tapping of metals. Additives which contain sulfur either in free form or in loosely bound form, principally made by sulfurizing a fatty body or fatty oil with or without subsequent phosphorizing the sulfurized product so produced, are among the principal ingredients used for this purpose. The incorporation of small amounts of fatty oil and sulfur in lubricating oils to compound an extreme pressure lubricant does not always result in a finished product which is compatible under all conditions of use or storage or which exhibits the preferred characteristics of an extreme pressure lubricant. Often the addition of specialized additives for the purpose of adjustment of the final viscosity, stability, or appearance of the finished product upsets one or more of the other desirable physical properties or performance characteristics to the end that extreme pressure gear lubricants which do not exhibit these difficulties and which are more versatile, more easily manufactured, extremely stable during storage, and exhibit good performance characteristics at reduced cost are often very difficult to compound.

The invention comprises specifically the discovery of a formulation for extreme pressure lubricants which includes as a part thereof a sulfur and/or phosphorous carrier along with an extreme pressure additive of the chlorinated type incorporated in a mineral oil which overcomes the difficulties of incompatibility and storage stability while at the same time exhibits good performance characteristics. The extreme pressure lubricants of the present invention are characterized by their ease of manufacture and their ability to withstand the extreme conditions to which such lubricants are subjected in use.

Accordingly, the principal object of the present invention is to provide an extreme pressure lubricating composition including a sulfur and/or phosphorous carrier and an extreme pressure additive of the chlorinated type.

A second object of this invention is to provide an extreme pressure gear lubricant comprising a mineral oil, a sulfur and phosphorous carrier, and an extreme pressure additive of the chlorinated type.

A third object of this invention is to provide an extreme pressure gear lubricant composition including a sulfur carrier and a phosphorous carrier, a viscosity index improver, and a chlorinated high molecular weight extreme pressure additive.

2

The extreme pressure gear lubricants of the present invention comprise two components—first, an extreme pressure concentrate and, second, the mineral oil portion of the composition, principally a solvent refined Mid-Continent mineral oil. The extreme pressure concentrate is composed of a sulfur and phosphorous carrier and a chlorinated extreme pressure additive.

The sulfur and phosphorous carrier may comprise a sulfurized non-fat material, such as Metalyn; a phosphorized fatty oil, such as phosphorized glyceryl trioleate; a sulfurized and phosphorized fatty oil, such as sulfurized-phosphorized lard oil; sulfurized mineral oils; sulfurized alkyl esters of animal and vegetable fatty acids where the alkyl group comprises methyl, ethyl, propyl or butyl groups; and combinations of these sulfur-containing constituents alone or in solution in an oleaginous substance. For example, the reaction product of petroleum and fatty oils and a phosphorous-containing material prepared in accordance with United States Patent 2,142,998 may be used. The sulfurized-phosphorized base described in United States Patent 2,211,306 is an excellent extreme pressure lubricant base for use in accordance with this invention. Many of these sulfurized and/or phosphorized bases are expensive and difficult to compound into a compatible composition. A particularly useful combination of extreme pressure bases to be used in accordance with this invention comprises sulfurized Metalyn and phosphorized glyceryl trioleate. In particular this combination along with the chlorinated extreme pressure agents has been found to be a suitable substitute for such more expensive and difficult compounded bases as dibenzyl disulfide in extreme pressure compositions.

The Metalyn referred to above is a trade name for methyl esters of tall oil, and it is prepared by the methyl esterification of tall oil acids under elevated pressure followed by distillation of the ester. This product, now being manufactured by the Hercules Powder Company, will have the following characteristics:

|                                               |      |                                   |
|-----------------------------------------------|------|-----------------------------------|
| Percent methyl esters of rosin acids          | 45.0 | (typical).                        |
| Percent methyl esters of fatty acids          | 47.0 | (typical).                        |
| Percent unsaponifiable modified AOCS          |      |                                   |
| Ca 6b-40                                      |      | 8.0 max.                          |
| Saponification No. (drastic, Hercules method) |      | 155/170.                          |
| Acid No. (AOCS Da 14-42)                      |      | 5.0 max.                          |
| Iodine No. (AOCS Cd 1-25)                     |      | 120/130.                          |
| Acetyl value (AOCS Cd 4-40)                   |      | 10.0 max.                         |
| Color (Gardner 1933)                          |      | 12.0 max.                         |
| Specific gravity 20°/20° C.                   |      | .95/.975.                         |
| Flash point °C. (COC)                         |      | 182° min.                         |
| Freezing point °C.                            |      | 10.0 max.                         |
| Viscosity at 100° F. SUS (ASTM D4445-46T)     |      | 70/100.                           |
| Moisture (AOCS Ca 2a-5)                       |      | 0.1 max.                          |
| Appearance at 20°/30° C.                      |      | Clear and free of foreign matter. |

In sulfurizing the Metalyn, elemental sulfur in the form of finely powdered flowers of sulfur is sifted in small increments into a kettle containing the Metalyn heated to about 275° to 285° F., while being vigorously agitated by a mechanical agitator. Although it is preferred to react 93 parts of Metalyn with 7 parts by weight of sulfur, the ratio of Metalyn to sulfur may suitably vary from about 85 parts Metalyn—15 parts sulfur to 97 parts Metalyn—3 parts sulfur.

After the addition of the sulfur to the Metalyn is completed, the temperature of the mixture is raised to 350° F. During the initial stages of the sulfurization reaction, it is important to keep the temperature about 20° to 30° below the flash point of Metalyn (385° F.). Reaction

is allowed to proceed for approximately 7 to 8 hours when it should be complete as indicated by a copper strip test. Shorter reaction periods are possible where efficiently heated kettles are available. During the final stages of the reaction, the temperature may be allowed to rise to 375° F. to insure complete reaction. The end of the reaction is determined by immersing a polished copper strip in a sample of the product for one minute at 300° F. If the copper strip remains bright, the reaction is completed. As previously pointed out, mechanical agitation and not air-blowing is used during the entire reaction period. The finished reaction product will have the following characteristics:

|                          |      |
|--------------------------|------|
| API gravity              | 8.0  |
| Lbs. per gallon          | 8.45 |
| Percent sulfur           | 6.26 |
| SUS viscosity at 210° F. | 56.2 |

Although this is the preferred product, it will be understood that the sulfurized Metalyn may contain from approximately 3 to 10 percent of sulfur. Where smaller amounts of sulfur are used, the reaction time and/or temperature may be reduced. Similarly, where larger amounts of sulfur are used, longer reaction times will be required in order to obtain a finished product. Higher temperatures will hasten the reaction time, but temperatures in excess of 400° F. should be avoided.

It will be understood that other esters of tall oil acids such as the ethyl, propyl, butyl, and amyl may be sulfurized in the same manner as Metalyn to form one constituent of the E. P. base. If desired mixtures of the several esters may be used instead of a single ester in order to obtain desired viscosity, pour point and other properties in the finished oil. The ethylene, propylene and butylene glycol dioleates may also be used.

In preparing phosphorized glyceryl trioleate, it is preferred to use glyceryl trioleate having the following specifications:

|                        |                                                      |
|------------------------|------------------------------------------------------|
| Acid No                | 10.0 max.                                            |
| Saponification No      | 187.0 min.                                           |
| Percent unsaponifiable | 3.5 max.                                             |
| Iodine value           | 75/85.                                               |
| Percent moisture       | 0.3 max.                                             |
| Acetyl value           | 40 max.                                              |
| Percent free glycerine | 0.25 max.                                            |
| Color                  | Water white to light amber.                          |
| Component fatty acids  | 80% oleic min.; 12% linoleic max.; 8% saturated max. |

Phosphorus sesquisulfide is used for phosphorization because of the uniformity of the resulting products. Other sulfides of phosphorus such as phosphorus pentasulfide, cause undesirable polymerization. It is important that a pure form of phosphorus sesquisulfide be used since impure material produces a dust-like sediment in the finished product. Pure phosphorus sesquisulfide has a uniformly light yellow color, while the impure material is characterized by small particles of grayish material running uniformly through the entire sample.

In the preparation, 195 parts by weight of glyceryl trioleate are heated in a kettle to 185° to 195° F. with vigorous mechanical agitation. To the heated material is added 5 parts by weight of finely powdered phosphorus sesquisulfide in small increments. When the total amount of phosphorus sesquisulfide is added, the temperature of the mixture is raised to 220° to 230° F. and the temperature maintained at this level until the reaction is complete, which should require about 4 to 5 hours. The completion of the reaction is determined by immersing a copper strip in a sample of reaction mixture at the temperature of 210° F. for 3 minutes. If the strip remains bright, the reaction is completed. During the entire reaction, mechanical agitation, and not air-blowing, is used. The finished phosphorized glyceryl trioleate will have the following characteristics:

|                           |      |
|---------------------------|------|
| API gravity               | 19.7 |
| Lbs. per gallon           | 7.79 |
| Weight percent sulfur     | 0.97 |
| Weight percent phosphorus | 1.26 |
| SUS viscosity at 210° F.  | 67.7 |

The chlorinated extreme pressure additive may include any chlorinated hydrocarbon, naphthalene compound, paraffin compound, or wax compound, such as chlorinated naphthalenes, known under the trade names of Halowax 1020 and Halowax 1014, or combinations of chlorinated naphthalene and chlorinated paraffins, known under the trade name of Chlorowax 40. These chlorinated derivatives of naphthalene may contain from 10 to 40 percent of chlorine. Other chlorinated ring and chain compounds may be used, including chlorinated petroleum wax, chlorinated aliphatic hydrocarbons, and alpha-chlornaphthalene.

Various other additives may be incorporated including, for example, pour point depressants, anti-corrosive compounds, other extreme pressure additives, viscosity index improvers, solubilizers, etc. One particularly advantageous additive comprises a viscosity index improver, such as the proprietary product known as Acryloid 150, which product comprises a pour depressant for the oil and is available commercially as a polymeric fluid. Chemically, this product is a methyl methacrylate polymer having the following properties: specific gravity, 60/60, 0.89; viscosity at 210° F., 3100 SUS; viscosity at 100° F., 27,500 SUS.

The mineral oil portion of the composition may comprise any lubricating oil or refined fractions thereof. The combination of a 150 viscosity bright stock and 170 viscosity neutral of the high V. I. type has been found particularly useful in preparing gear oil lubricants in accordance with this invention. The bright stock and neutral are proportioned to give a final viscosity to the finished lubricant in the range of 80-90 SUS at 210° F. All components of the gear oil composition may be blended together at temperatures from 185° to 195° F. The blending may take place in short periods of 15 to 30 minutes to produce a stable satisfactory gear lubricant. The following examples are given as typical formulations representing combinations of preferred sulfur carriers, chlorinated compounds, and other additives:

(1)

(Percent by weight composition)

|       |        |                                                                                                                 |
|-------|--------|-----------------------------------------------------------------------------------------------------------------|
| 50    | 13.0%  | (5.0 sulfurized Metalyn—10.8 wt. percent of total; 1.0 phosphorized glyceryl trioleate—2.2 wt. percent of total |
| 55    | 0.3%   | Halowax 1020                                                                                                    |
|       | 0.5%   | Acryloid 150                                                                                                    |
| 59.0% | 59.0%  | 150 vis. Mid-Continent solvent refined bright stock                                                             |
| 60    | 27.2%  | 170 vis. Mid-Continent solvent refined neutral                                                                  |
|       | 100.0% | total                                                                                                           |

(2)

|    |        |                                                                                                               |
|----|--------|---------------------------------------------------------------------------------------------------------------|
| 65 | 10.0%  | 3.0 sulfurized Metalyn—7.5 wt. percent of total; 1.0 phosphorized glyceryl trioleate—2.5 wt. percent of total |
| 70 | 0.2%   | 10.0 Halowax 1020, 0.11 wt. percent of total; 1.0 Chlorowax 40, 0.09 wt. percent of total                     |
| 70 | 1.0%   | Acryloid 150                                                                                                  |
| 75 | 55.0%  | 150 vis. Mid-Continent solvent refined bright stock                                                           |
| 75 | 33.8%  | 170 vis. Mid-Continent solvent refined neutral                                                                |
|    | 100.0% | total                                                                                                         |

|                                                           |  |
|-----------------------------------------------------------|--|
| 12.0% sulfurized and phosphorized lard oil                |  |
| 0.3% Halowax 1020                                         |  |
| 0.5% Acryloid 150                                         |  |
| 21.0% 150 vis. Mid-Continent solvent refined bright stock |  |
| 21.0% extract from 150 vis. bright stock (Mid-Continent)  |  |
| 45.2% 170 vis. Mid-Continent solvent refined neutral      |  |
| 100.0% total                                              |  |

The physical and chemical characteristics of the components used in blending 90 grade extreme pressure lubricants are shown in Table I:

termine the storage stability or compatibility of Halowaxes with extreme pressure concentrates. The compositions tested were prepared by adding different amounts of Halowax 1014 and Halowax 1020 to sulfurized Metalyn, phosphorized glyceryl trioleate, and a mixture composed of sulfurized Metalyn and phosphorized glyceryl trioleate extreme pressure base. These concentrates were prepared by heating the extreme pressure compound to 220-230° F. and subsequently adding the Halowaxes with vigorous stirring. The blends were stirred until cooled to about 150-160° F. Storage tests conducted under these conditions of high concentration are much more indicative of stability of the products than tests conducted in

TABLE I  
*Characteristics of the components used blending the 90 grade E. P. lubes*

|                         | API<br>grav. | Flask,<br>° F. | Fire,<br>° F. | Viscosities, ° F., SUS |       |       | V. I. | Pour<br>° F. | Per-<br>cent<br>S | Per-<br>cent<br>P | Flow<br>pt.<br>° C. | Color                | Per-<br>cent<br>Cl | Sp. gr.,<br>25° C.     |
|-------------------------|--------------|----------------|---------------|------------------------|-------|-------|-------|--------------|-------------------|-------------------|---------------------|----------------------|--------------------|------------------------|
|                         |              |                |               | 100                    | 130   | 210   |       |              |                   |                   |                     |                      |                    |                        |
| Halowax 1020            |              |                |               |                        |       |       |       |              |                   |                   |                     |                      |                    |                        |
| Halowax 1014            |              |                |               |                        |       |       |       |              |                   |                   |                     |                      |                    |                        |
| S-P lard oil            |              |                |               |                        |       |       |       |              |                   |                   |                     |                      |                    |                        |
| Extract from brt. stock | 13.2         | 380            | 445           | 25,000 ext.            | 4,894 | 525   | 9     | +80          | 2.29              | 0.245             | 116-120<br>277-283  | Light<br>Pale yellow | 53.3<br>56.5       | 1.69-1.74<br>1.76-1.88 |
| 150 vis. brt. stock     | 26.4         | 570            | 630           | 2,365                  | 897   | 150.8 | 100   | 0            | 0.48              |                   |                     |                      |                    |                        |
| 170 vis. neutral        | 28.2         | 415            | 480           | 2,379                  | 882   | 146.8 | 96    | +5           | 0.56              |                   |                     |                      |                    |                        |
|                         |              |                |               |                        | 94.6  | 44.9  | 103   | 0            | 0.18              |                   |                     |                      |                    |                        |

In Table II a comparison is made of extreme pressure compositions (Example 1) containing a sulfurized-phos-

which mineral oil is part of the composition. The results are shown in Table III.

TABLE II  
*Determination of optimum concentration of halowaxes in 80/90 grade E. P. lubes by modified SAE and Timken bench test*

| Blend                                             | 1      | 2      | 3      | 4      | 5      | 6      | 7      | 8      | 9      | 10     |
|---------------------------------------------------|--------|--------|--------|--------|--------|--------|--------|--------|--------|--------|
| Percent by weight composition met./GTO E. P. base |        | 13.0   | 13.0   | 13.0   | 13.0   | 13.0   | 13.00  | 13.00  | 13.0   | 13.0   |
| Dibenzyl disulfide                                | 1.0    | 1.0    |        |        |        |        |        |        |        | 1.0    |
| S-P lard oil                                      | 12.0   |        |        |        |        |        |        |        |        |        |
| Halowax 1020                                      |        |        |        | 0.3    | 0.4    | 0.5    |        |        |        |        |
| Halowax 1014                                      |        |        |        |        |        |        |        |        |        |        |
| Acryloid 150                                      | 0.5    | 0.5    | 0.5    | 0.5    | 0.5    | 0.5    | 0.25   | 0.35   | 0.5    |        |
| Extract from brt. stck                            | 21.0   |        |        |        |        |        |        |        |        |        |
| 150 bright stock                                  | 17.0   | 59.0   | 59.0   | 59.0   | 59.0   | 59.0   | 59.00  | 59.00  | 59.0   | 59.0   |
| 170 neutral                                       | 48.5   | 26.5   | 27.5   | 27.2   | 27.1   | 27.0   | 27.25  | 27.15  | 27.0   | 26.5   |
| Viscosity (SUS):                                  |        |        |        |        |        |        |        |        |        |        |
| 210° F.                                           | 84.5   | 84.5   | 86.0   | 85.9   | 85.9   | 85.6   | 85.7   | 85.5   | 85.9   | 88.4   |
| 130° F.                                           |        | 363    | 377    | 376    | 378    | 376    | 376    | 378    | 378    | 254    |
| 100° F.                                           |        | 821    | 840    | 875    | 879    | 874    | 876    | 876    | 886    | 819    |
| Viscosity index                                   | 106    | 104    | 103    | 103    | 103    | 102    | 103    | 102    | 102    | 104    |
| Timken, 800 R. P. M.:                             |        |        |        |        |        |        |        |        |        |        |
| Beam load (lbs.)                                  | 59     | 51     | 59     | 51     | 59     | 51     | 33     | 59     | 59     | 51     |
| Pressure (p. s. i.)                               | 32,000 | 37,750 | 41,450 | 33,250 | 37,750 | 31,700 | 19,000 | 36,300 | 37,575 | 32,400 |
| Modified SAE:                                     |        |        |        |        |        |        |        |        |        |        |
| Weight loss                                       | Mg     | 19     | 32.8   | 29.4   | 21.1   | 32.7   | 22.9   | 24.6   | 26.1   | 30.5   |
| Ring appearance                                   | OK     | OK     | OK     | OK     | OK     | OK     | OK     | OK     | OK     | OK     |

phorized lard oil and Acryloid 150 and (Example 2) containing dibenzyl disulfide in addition to the extreme pressure base as exemplary of products which meet the viscosity, V. I., Timken, and Modified SAE tests. Example 3 shows a composition wherein the sulfur-containing carrier is a sulfurized Metalyn-phosphorized glyceryl trioleate extreme pressure base giving acceptable viscosity, V. I., Timken, and modified SAE tests. Examples 4 through 9 show compositions including chlorinated extreme pressure additives in accordance with this invention which meet the physical requirements of extreme pressure lubricants. In order to further demonstrate the present invention, a series of tests were conducted to de. 75

TABLE III  
*Compatibility of Halowaxes with E. P. concentrates*

| Blend                        | 11    | 12    | 13    | 14    | 15   | 16   |
|------------------------------|-------|-------|-------|-------|------|------|
| Parts by weight composition: |       |       |       |       |      |      |
| Halowax 1014                 | 0.5   |       | 0.037 |       | 0.5  |      |
| Halowax 1020                 |       | 0.5   |       | 0.037 |      | 0.5  |
| Sulfurized Metalyn           | 5.0   | 5.0   |       |       |      |      |
| Phosphorized GTO             |       |       | 1.0   | 1.0   |      |      |
| Metalsyn/GTO E. P. base      |       |       |       |       | 13.0 | 13.0 |
| Storage stability, 60 days:  |       |       |       |       |      |      |
| ET                           | OK    | OK    | OK    | OK    | OK   | OK   |
| 32° F.                       | Solid | Solid | Solid | Solid | OK   | OK   |

The Halowaxes may be incorporated in concentrations from 0.3 weight percent to 9.0 weight percent to form compatible mixtures with the sulfur-phosphorous extreme pressure base. The Halowaxes may be present in concentrations ranging from 0.3 to 0.5 weight percent of finished product including the mineral oil carrier.

The proportions of ingredients used in compositions prepared in accordance with the present invention may vary somewhat from the exact weight percent compositions shown in the examples. The sulfurized and/or phosphorized extreme pressure base may be present in from about 10 to 13 weight percent. The amount of viscosity index improver represented by Acryloid 150 may vary from 0.4 to 1.5 weight percent depending on the amount required to bring the composition to the desired viscosity index. Further the percent of chlorinated extreme pressure compound may vary from about 0.1 to 0.3 weight percent or as high as 0.5 weight percent. The mineral oil can make up the balance of the composition. One advantage of the invention is that by substituting the chlorinated compounds for the dibenzyl disulfide, a composition can be prepared with less cost and by using less materials. Furthermore, the difficulties in handling and compounding dibenzyl disulfide are avoided.

What is claimed is:

1. A lubricant additive consisting of a mixture of about 3-5 parts by weight of sulfurized methyl esters of tall oil acids, said sulfurized product containing about 3% to 10% by weight of sulfur acid being obtained by the reaction of methyl esters of tall oil acids with elemental sulfur at a temperature 20-30° F. below the flash point of said esters until a product is obtained which is non-corrosive to a polished copper strip when in contact therewith for about one minute at a temperature of 300° F., about 1 part by weight of phosphorized glyceryl trioleate, said phosphorized product containing about 0.97 weight percent of sulfur acid about 1.26 weight percent of phosphorus and being obtained by reacting glyceryl trioleate with phosphorus sesquisulfide at a temperature of about 220° to 230° F. until a product is obtained which is non-corrosive to a polished copper strip when in contact therewith for about three minutes at a temperature of 210° F., and about 0.1 to 0.5 part by weight of a chlorinated naphthalene containing about 10 to 40% by weight of chlorine, said mixture being characterized by its stability during storage at room temperatures and at a temperature of 32° F.

2. A lubricant additive consisting of a mixture of about 13.0 parts by weight of a sulfur- and phosphorus-containing base consisting of about 5.0 parts of sulfurized methyl esters of tall oil acids containing about 6.26 weight percent of sulfur and being obtained by the reaction of said methyl esters of tall oil acids with elemental sulfur at a temperature of 20-30° F. below the flash point of

said esters until a product is obtained which is non-corrosive to a polished copper strip when in contact therewith for about one minute at a temperature of 300° F., about 1.0 part by weight of phosphorized glyceryl trioleate, said phosphorized product containing about 0.97 weight percent of sulfur and about 1.26 weight percent of phosphorus sesquisulfide at a temperature of about 220° to 230° F. until a product is obtained which is non-corrosive to a polished copper strip when in contact therewith for about three minutes at 210° F. and about 0.5 parts by weight of a chlorinated naphthalene containing about 10% to 40% by weight of chlorine, said mixture being characterized by its stability during storage at room temperature and at a temperature of 32° F.

3. An extreme pressure lubricant composition consisting of about 59.0 weight percent of 150 vis. Mid-Continent solvent refined bright stock, about 27.2 weight percent of 170 vis. Mid-Continent solvent-refined neutral, about 13.0 weight percent of an extreme pressure base consisting of a mixture about 5.0 parts by weight of sulfurized methyl esters of tall oil acids containing about 6.26 weight percent of sulfur and being obtained by the reaction of said methyl esters of tall oil acids with elemental sulfur at a temperature 20° to 30° F. below the flash point of said esters until a product is obtained which is non-corrosive to a polished copper strip when in contact therewith for about one minute at a temperature of 300° F., and about 1.0 part by weight of phosphorized glyceryl trioleate, said phosphorized product containing about 0.97 weight percent of sulfur and about 1.26 weight percent of phosphorus and being obtained by reacting glyceryl trioleate with phosphorus sesquisulfide at a temperature of about 220° to 230° F. until a product is obtained which is non-corrosive to a polished copper strip when in contact therewith for about three minutes at 210° F. and 0.3 part by weight of a chlorinated naphthalene containing about 10% to 40% by weight of chlorine and about 0.5 part by weight of methyl methacrylate having a viscosity at 210° F. of 3100 SUS and a viscosity of 100° F. of 27,500 SUS, said lubricant composition being characterized by its storage stability and ability to pass the Timken and Modified SAE tests.

#### References Cited in the file of this patent

#### UNITED STATES PATENTS

|           |                |                |
|-----------|----------------|----------------|
| 2,204,538 | Lincoln        | June 11, 1940  |
| 2,242,260 | Prutton        | May 20, 1941   |
| 2,254,337 | Whittier       | Sept. 2, 1941  |
| 2,268,608 | McNulty et al. | Jan. 6, 1942   |
| 2,407,954 | Fenske         | Sept. 17, 1946 |
| 2,468,520 | Sproule et al. | Apr. 26, 1949  |
| 2,592,497 | Waddey et al.  | Apr. 8, 1952   |
| 2,644,810 | Beretyas       | July 7, 1953   |

UNITED STATES PATENT OFFICE  
CERTIFICATE OF CORRECTION

Patent No. 2,830,024

April 8, 1958

Paul R. Chapman et al.

It is hereby certified that error appears in the printed specification of the above numbered patent requiring correction and that the said Letters Patent should read as corrected below.

Column 1, line 23, for "resstance" read -- resistance --; line 25, for "owrking" read -- working --; column 2, line 8, for "carried" read -- carrier --; line 38, for "Sompany" read -- Company --; line 55, for the designation "D4445" read -- D445 --; column 6, lines 5 and 6, for "composing" read -- comprising --; columns 5 and 6, Table II, under the column headed "7", opposite "Pressure (p.s.i.)" for "19.000" read -- 19,000 --.

Signed and sealed this 27th day of May 1958.

(SEAL)

Attest:

KARL H. AXLINE

Attesting Officer

ROBERT C. WATSON  
Commissioner of Patents